

Jan. 28, 1941.

H. J. NESS

2,229,667

SILVER-LEAD ALLOY

Filed April 30, 1938

2 Sheets-Sheet 1

*Fig. 1*



*Fig. 2*



*Fig. 3*



Inventor  
Harold J. Ness  
BY

*M. J. Reynolds*  
Attorney

Jan. 28, 1941.

H. J. NESS

2,229,667

SILVER-LEAD ALLOY

Filed April 30, 1938

2 Sheets-Sheet 2

*Fig. 4*



INVENTOR

Harold J. Ness

BY

M. J. Reynolds  
ATTORNEY

## UNITED STATES PATENT OFFICE

2,229,667

## SILVER-LEAD ALLOY

Harold J. Ness, Bloomfield, N. J.

Application April 30, 1938, Serial No. 205,391

17 Claims. (Cl. 75—167)

This invention relates to alloys and to the method of producing the same, and more particularly to bearing metal alloys composed primarily of silver and lead.

5 In the development of greater power and higher speeds in internal combustion engines for automobile and aircraft and in other machines, it has been necessary to employ bearing alloys which, at the elevated temperatures obtained

10 in such machines, have mechanical properties, such as compressive strength, tensile strength and resistance to pounding, exceeding those of the usual white-metal bearing alloys. Alloys of copper and lead have been employed to some extent to replace tin-base alloys for such service.

In a copending application Serial No. 193,277, filed March 1, 1938, I have disclosed a method of producing copper-lead alloys by which up to 70% lead may be finely divided and evenly dispersed 20 in copper. Copper, however, by itself is not a good bearing metal. Silver, while not satisfactory by itself, as a bearing metal, has bearing properties far superior to copper. Since, however, the solubility of lead in silver in the solid 25 state is negligible, it has not been possible, heretofore, to incorporate more than about 4% of lead in silver. Any additional lead added to the silver merely segregates in relatively large masses in the silver.

30 One of the objects of the present invention is to eliminate the difficulties which have heretofore accompanied the production of such silver-lead alloys.

Another object is to provide a method of producing silver-lead alloys in which agitation of the molten mass is obtained without mechanical stirring.

Another object is to provide such a method in which the agitation of the mass continues in the 40 mold and up to the time of solidification of the mass.

Another object is to provide a method of making silver-lead alloys in which the lead will be firmly bonded to the silver and retained in a 45 finely divided state in a continuous network or matrix of the silver.

Still another object is to provide such a method which will result in a uniform dispersion and fine subdivision of lead in silver.

50 Another object is to provide a process of making silver-lead alloys of high physical properties.

Still another object is to provide a method of producing silver-lead alloys free from segregation, having much greater lead content than has 55 heretofore been possible.

Another object is to provide a simple, economical and reliable method of producing silver-lead alloys.

A still further object is to produce a silver-lead 60 alloy of strong physical properties and high anti-

friction and anti-scoring properties at either low or elevated temperatures.

Another object is to provide a silver-lead bearing metal alloy in which sweating out of the lead at high operating temperatures and/or pressures will not occur. 5

Another object is to produce silver-lead alloys having lead contents up to 70% or more.

Another object is to produce an oxygen free 10 alloy of silver and lead.

Another object is to produce silver-lead alloys in which the lead is contained within the grain boundaries of the silver.

Another object is to provide a process of making silver alloys in which the molten alloy will 15 be free from dross.

Other objects and advantages will hereinafter appear.

The present invention is based, in part, upon the discovery that when lithium is introduced 20 into a silver-lead alloy, and precautions are observed to maintain some lithium in the alloy, a natural circulation or agitation of the molten mass occurs which enhances the intimate mixing of the alloying ingredients and that such 25 agitation or automatic stirring action continues, after it has once started, until actual solidification of the alloy upon cooling. As a consequence, no opportunity is afforded for the ingredients to segregate. Moreover, the agitation is very rapid, 30 apparently occurring simultaneously throughout the entire molten mass so that a thorough stirring of the molten mass results and, upon solidification thereof, the lead of the alloy is retained in a uniform and finely subdivided form within a 35 silver matrix and is intimately bonded thereto.

The lithium, when maintained in a small proportion in the silver-lead mixture by regulated conditions of operation, the nature of which will 40 hereinafter appear, produces in the molten mass as the temperature thereof is raised to above a certain temperature, a violent agitation which is accompanied by considerable surface turbulence and a crackling and simmering sound. The temperature at which this agitation commences 45 varies with the proportion of the silver and lead in the mixture and is readily determined, for any particular mixture, from observation of the surface of the mass, since the agitation of the mass is pronounced and unmistakable. The proportion of lithium required to effect this stirring or 50 agitating action is very small, very definite and active agitation and uniform and fine dispersion of the lead having been obtained in the production of silver-lead alloys, which upon analysis 55 showed only a trace of lithium.

The lithium may be introduced into the mixture in a variety of ways, as for example, alloyed with the lead, alloyed with the silver, in a solid metallic state either alone or wrapped in other 60

metals, such as silver, copper, lead, etc., or as a vapor.

While the method of introducing lithium into the molten mass as an alloy of either lead or silver is highly satisfactory, this is not necessary since the pure lithium may be added directly to the fused mixture of lead and silver, either by dropping solid pieces of lithium therein or by packing it in a crucible which is inverted and 10 pushed down into the molten mass.

Since the quantity of lithium required is extremely small, it may be added as a vapor, merely by creating a lithium vapor or atmosphere about the crucible, in any suitable manner, as 15 for instance, by liberation of lithium from the lining of a furnace, which has been previously treated with lithium, as will hereinafter appear, or by introducing lithium metal or a compound thereof into the furnace atmosphere. The pouring 20 may be done as soon as the agitation begins, although the quality and fineness of dispersion is not affected by continued heating since no dross occurs, even at high temperatures. Due to the inherent agitation of the molten mass with 25 continued heating thereof, it may be readily cast from holding furnaces, which are generally used when producing die or permanent mold castings.

The molten mass, as it cools in the molds, continues to agitate until stopped by solidification 30 thereof. There is, therefore, no opportunity for segregation of either the lead or silver to occur. The molten mass is very dense and therefore there is little or no shrinkage during solidification.

35 It has been found, however, that the mere addition of lithium to the charge does not result in the stirring action described nor in the production of a fine grain and uniformly distributed structure, but in addition it is necessary to prevent, at least in part, loss of lithium from the charge or to conduct the process under conditions which will supply additional lithium to the charge as the process continues. In practice it has been found that the linings of the furnaces used, which contain large proportions of silica, 40 unless pretreated react with the lithium of the charge, as a result of which the lithium is very quickly and completely absorbed from the charge. In order to prevent the loss of the lithium from the charge in this manner and to provide continuously a lithium coating atmosphere about the crucible during heating of the charge, the lining of the furnace is treated with lithium vapor at a high temperature so that the lining 45 will take up a portion of the lithium with which it is treated. The furnace linings thus treated will remain in a suitable lithiated condition for a considerable period, when not in use, and may be used for melting lithium containing silver 50 alloys repeatedly without reconditioning. This conditioning of the furnace lining, it is believed, results in a saturation or near saturation of the lining by the lithium or a compound thereof whereby the lining, upon subsequent melting of a charge, is not free to readily absorb additional 55 lithium from the charge, but on the contrary liberates lithium to produce a lithium containing atmosphere over and possibly through the crucible, which atmosphere retards the escape of 60 lithium from the charge. If desired, this lithium containing atmosphere may comprise the sole means of introducing the lithium into the charge, excellent results being obtainable by merely heating a pure silver and lead mixture in a furnace 65 having a lithium treated lining. Sufficient 70

lithium is absorbed into the charge, from the lithium containing atmosphere produced from heating of the lining, to cause pronounced agitation of the molten mass and a fine and uniform distribution of the lead in the silver upon casting. 5 This method of introducing the lithium into the melt is, in some respects, a preferred one since in the resulting castings the lead is extremely well distributed and finely divided.

The amount of lead which may be combined 10 with silver while retained in a uniformly dispersed and finely divided state therein may vary up to about 70% lead or even higher. When silver, lead and lithium alone are employed or even if small amounts of such metals as tin, copper and 15 zinc are added, the silver or silver and other alloying components, if present, form a continuous matrix or cellular network in which the lead is dispersed as discontinuous finely divided particles, firmly bonded to the silver, a condition which produces high tensile and compressive 20 strength and resistance to pounding. The grain structure of the silver-lead alloys produced in accordance with the process herein described assumes the grain structure of oxygen free silver 25 with the lead finely divided and highly dispersed within the individual silver grains, each silver grain including a countless number of separate lead particles. The alloy being produced in a lithium containing atmosphere, it is completely 30 oxygen free and has not only grain formation but physical properties comparable to oxygen free silver.

The number of lead particles appearing in a cross section of the silver-lead alloy of the present invention is enormous and for an alloy containing 40% lead, it may vary from, say, 50,000 to several hundred thousand per square inch and the average size of a lead particle may be of the order of magnitude of  $10^{-6}$  square inches or smaller although the present invention is not limited to such particle size or distribution range, the foregoing figures being given only by way of example. The presence of lithium in the alloy in addition to its dispersing action, toughens and 45 strengthens both the silver and lead of the alloy and increases their tensile strength, thereby further enhancing the physical properties of the alloy. Moreover, due to the encasement of the individual lead particles within the silver grains, 50 the lead will not sweat out under operating conditions and temperatures. The addition of copper, tin and/or zinc in small percentages serves to harden the alloy.

The dispersion of the lead in the silver is extremely uniform and finely divided whether the casting is permitted to cool fast or slowly and therefore it may be readily cast in steel, iron or dry sand molds. The sand employed should be substantially chemically inert to lithium. With 60 the present process the pouring can be conducted directly through the air without oxygen absorption due to the presence of the lithium in the melt, which appears to form a protective atmosphere about the molten stream.

In order that the invention may be more clearly understood reference will now be had to the accompanying drawings, in which:

Fig. 1 is a vertical section of a gas fired furnace suitable for the production of a silver-lead-lithium alloy;

Fig. 2 is a photomicrograph of a silver-lead-lithium alloy containing substantially 10% lead and less than 1% of lithium, with the remainder silver X100;

Fig. 3 is a photomicrograph of a silver-lead-lithium alloy containing substantially 70% lead and less than 1% of lithium, with the remainder silver X100; and

5 Fig. 4 shows means for introducing lithium compounds into the furnace of Fig. 1.

Referring to Fig. 1, I have shown a gas fired furnace of conventional construction having a refractory lining 10 within which is contained a crucible 11, which may be of graphite, preferably lined with a refractory cement such as sillimanite to prevent reaction of the lithium therewith. A refractory cover plate 12 having a suitable gas vent 13 is provided. Gas and air are admitted 15 through a burner ring 14 surrounding the furnace, the gas being supplied through a conduit 15 and the air through a conduit 16. A blower 17, shown diagrammatically, and suitable valves (not shown) control the amount of air and gas supplied. In order to assist in maintaining an adequate supply of lithium vapor in the furnace above and around the crucible, the incoming air is caused to flow through a chamber 18 containing 20 solid lithium particles or a powdered compound of lithium, contained between metal screens 19. A bypass sleeve 20 permits air to be introduced independently of the lithium chamber 18, if desired. Sufficient lithium either in elemental or oxide form is carried into the furnace 25 with the air and vaporized therein, to produce a strong lithium spectral line when the gases escaping from the furnace are viewed with a spectroscope, thus denoting the presence of lithium in the furnace gases in an elemental form and in an ionized condition. Experimental data indicates that the presence of lithium in the elemental form is due, at least in part, to the reducing action of carbon monoxide gas in the furnace on lithium oxide, under the conditions prevailing in 30 the furnace. A furnace lining which has been found suitable consists of silica 65%, alumina 25%, and the remainder ignition loss, i. e., moisture and other volatile material, and small percentages of iron, titanium, lime and magnesia.

45 The lining is treated by heating lithium in the furnace for a substantial period at a temperature sufficient to cause formation of a strong lithium vapor in the furnace as previously described. The lithium for treating the lining may be introduced into the furnace, as a charge, through the top thereof, although sufficient lithium can be carried into the furnace with the air flowing through the chamber 18, to effectively treat the lining. The sufficiency of the amount 50 of lithium or lithium compound taken up by the lining can be determined by melting a charge of silver and lead therein. If upon melting of such a charge an agitation of the mass occurs, the lining is sufficiently treated for a successful carrying out of the present process. If no agitation occurs, it is necessary to retreat the furnace lining in the same manner. The treatment can also be effected by applying to the lining a compound 55 of lithium, such as lithium chloride, thereon. The compound may be applied as a water solution or suspended or dissolved in other volatile vehicles, as fully set forth in my co-pending application Serial No. 112,988, filed November 27, 1936, and entitled "Furnaces."

70 In the process of producing silver-lead-lithium alloys in which the lithium is introduced into the furnace atmosphere from the lining of the furnace, it is desirable to replace or add to the lithium given off by the walls, by permitting a small amount thereof to be carried in by the air flow-

ing through the lithium containing chamber 18, although this is not necessary since repeated heats can be made with a single treatment of the furnace lining.

As previously stated, the charge is heated in 5 the lithium vapor containing atmosphere until circulation occurs after which it may be poured immediately or the heating may be continued for long periods until it is convenient or desirable to pour. 10

The alloy may be used for coating backing strips, such as steel, in the same manner disclosed for coating such strips with a copper-lead alloy in my copending application Serial No. 193,278 filed March 1, 1938. 15

Referring next to Figs. 2 and 3 of the drawings, it will be noted that the lead, indicated by the dark areas, is dispersed very uniformly throughout the silver and is in an extremely fine state of subdivision, whether the lead is present in a 20 low percentage (10% in Fig. 2) or a high percentage (70% in Fig. 3). The dark or lead particles, it will be noted, are extremely fine, substantially uniformly distributed and entirely surrounded by the silver, thus indicating a continuous 25 silver matrix with the lead particles dispersed directly in the silver grains.

As previously stated, the composition of the silver and lead content of the alloy may vary within wide limits while maintaining the advantages of fine structure and uniform dispersion. The relative amounts of lead and silver will be varied in accordance with the service to be performed by the alloy. 30

It is believed that the active portion of the 35 furnace atmosphere consists of lithium in the metallic state and that the lithium in the silver-lead alloy is also in a metallic state although these facts are difficult of determination and it is possible that under the conditions prevailing 40 in the furnace some active compound of lithium may be formed which effects the stirring action and imparts other beneficial characteristics to the alloy. The term "lithium" is employed in the claims, therefore, to include either metallic lithium or lithium in whatever other form it may occur in the furnace atmosphere and in the alloy. 45

In place of introducing metallic lithium into the furnace, a compound thereof, such as the chloride, fluoride, hydroxide, oxide, or carbonate 50 of lithium, or lithium containing ores such as spodumene or amblygonite, or mixtures thereof, may be used. The lithiated atmosphere may be provided in a gas fired furnace, for instance, by introducing a small quantity of a compound 55 of lithium in powdered form, into the air or gas stream leading into the furnace or it may be injected or blown directly into the furnace through an aperture provided in one of the walls thereof. An apparatus for introducing the powdered lithium compounds directly into the furnace or into the air or gas conduit extending 60 thereto is fully disclosed in my copending application Serial No. 143,410, filed May 19, 1937, and entitled "Injecting apparatus." In an oil 65 fired furnace the lithium compounds may be added directly to the oil, either as an oil soluble compound or in colloidal suspension. A process of treating fuel oil with lithium compounds is disclosed in my copending application Serial No. 70 154,203, filed July 17, 1937, and entitled "Promotion of combustion." In the case of electric furnaces the lithium compounds may be mixed with powdered carbon, such as graphite, and the mixture blown in a fine spray into the furnace in the 75

manner set forth in my copending application Serial No. 143,411, filed May 19, 1937, and entitled "Metallurgical process."

The amount of lithium compound required to produce the requisite condition of the furnace atmosphere is very small but is not critical and may be readily determined by experiment for any particular furnace. The furnace should be operated on the reducing side so that the furnace gases will contain a small percentage of carbon monoxide, the purpose of which will hereinafter appear. The desired rate or frequency of introduction of the lithium compound may be determined by spectroscopic examination of the gases escaping from the furnace.

The use of the lithium compounds in place of metallic lithium simplifies the problem of introducing the lithium into the furnace, since the suitable compounds are more stable and more readily handled. Moreover, such compounds are normally in a pulverulent state and the amount to be introduced can be readily metered and introduced by simple, reliable and inexpensive apparatus. Lithium metal, moreover, is several times as expensive as the compounds for equivalent amounts of lithium, since the metal must be produced from the compound by an expensive and involved process. Also, it has been found, when using a salt, such as lithium carbonate, introduced either continuously or at intervals throughout the process, that suitable results may be obtained in a new or unseasoned furnace, although with continued use a finer subdivision of the lead in the silver is obtained.

In Fig. 4 I have shown apparatus for continuously introducing lithium compounds into a melting furnace to provide a satisfactory atmosphere in which to produce a silver-lead alloy. In this figure the furnace is provided with a supply of a lithium compound, such as the carbonate, by an injecting apparatus comprising a cylindrical container 22 of transparent material, resting in a base casting 23 and having an upper closure member 24, both carried by a vertical support 25 mounted on a base 26. Extending into the chamber 22, through a stuffing gland 27, is a shaft 28 journaled in bearings 29 and 30. The shaft is revolved by a motor 31 through a belt 32. Mounted on the shaft 28 are several sets of blades 33a to 33e of decreasing length and increasing pitch. The lower blades 33a are integral with a collar 36 forming a labyrinth seal with a gland closure plate 35. A stack 36 extends downwardly from the top plate 24 and surrounds the upper blades 33e. When the container 22 is provided with a supply of a powdered lithium compound, the blades 33a to 33e agitate the compound, raising it in a cloud up through the stack 36, the powder then falling down around the outside of the stack.

A combustible mixture of air and gas under pressure is supplied by a blower 37 also driven by the motor 31 by a belt 38, the air and gas mixture being conducted by a conduit 39 into a gas cleaner 40 from whence the stream is diverted, part passing by conduit 41 into the base of the container 22, and part being conducted by conduit 42 to a Venturi nozzle 43, having communication with the container 22 by a conduit 44. The air and gas mixture directed into the container 22 becomes laden with the lithium compound as it passes through the container and is drawn out of the container by the jet 43 and directed into the furnace through the conduit 45. Suitable valves 46 and 47 in the

conduits 41 and 42 control the quantity of gas mixture and compound blown into the furnace. By supplying a gas and air mixture to the blower, the ratio of gas and air in the furnace is not disturbed by the fluid medium employed to convey the powders into the furnace. In place of the mixture of air and gas, either air alone or gas alone may be employed to convey the powdered compound into the furnace, although the use of air alone tends to create localized hot zones in the furnace and somewhat detracts from the efficiency of the action of the lithium compound in such zones. Excessive moisture in the air, such as results from high compression of the same, or in the gas employed, also detrimentally affects the action of the lithium compound and the maintenance of the proper lithiated atmosphere within the furnace, and should be avoided.

The lithium compound so introduced produces in the silver-lead charge a natural circulation or agitation of the molten mass in the same manner as does metallic lithium.

The furnace lining may be composed largely of silicon oxide and when such a lining is employed, the lithium compounds may be introduced into the furnace at spaced intervals since the lining serves as a storage and liberating medium whereby the desired atmosphere is maintained within the furnace between the periods of introduction of the lithium compound. It is not necessary, however, that the lining be of the particular composition specified heretofore, since linings have been found satisfactory having a silica content of about 31% with approximately 35 62% alumina and the remainder mainly iron oxide and titanium oxide. Linings of magnesium oxide, aluminum oxide and chromium oxide may also be employed or the furnace lining of hard burned brick of low permeability and low porosity containing approximately 50% silica and 44% alumina, having a bulk density of about 1.2 oz. per cu. inch and a fusion point of about 3200° F. A cement for bonding the bricks, such as sillimanite, cyanite, andalusite, and mullite, analyzing as follows: silica 38.07%, alumina 56.63%, titanium 1.14%, iron oxide .73%, ignition loss 2.78% and the remainder moisture and other impurities, has been found suitable. This cement may also be used as a coating for the bricks after 50 their assembly in the furnace. In general, cellular insulating brick or moulded or tamped-in linings have not been as satisfactory as linings built up from hard burned refractories, apparently due to the high permeability thereof or the 55 reaction of the lithium or one of its compounds with the binder employed in such moulded linings. Linings, hearths and other refractory parts of the furnace consisting of or containing silicon carbide have been found to react detrimentally 60 with the lithium of the atmosphere, due possibly to the nature of the binder commonly employed, causing breakdown of the refractory and to some extent, reduction in the efficiency of the lithium containing atmosphere for its intended purpose. 65

I prefer to introduce the lithium metal or compound into the furnace mixed with the air or fuel since this insures that it will pass through the hottest part of the flame, which is at a temperature several hundred degrees above the average furnace temperature. Hence the lithium or its compound will be more readily converted into a vapor.

Under the conditions prevailing in the furnace the lithium compound, or at least a por-

tion thereof, breaks down liberating free metallic lithium. The reaction is apparently first the formation of lithium oxide which reacts with carbon monoxide as follows:



The lithium is thus freed to combine with the oxygen of the furnace or any oxygen that may be included in the metal being heated and the 10 lithium carbonate of the above reaction is thermally broken down to lithium oxide liberating carbon dioxide. The reaction is then repeated with the lithium oxide so formed. As will be noted from the reactions set forth above each 15 particle of lithium present in the furnace goes through the above cycle repeatedly, until it ultimately escapes with the furnace gases and it is necessary, therefore, to supply additional lithium or lithium compounds only to replace 20 that so escaping and that deposited on the material being heated or on parts of the furnace.

In electric furnaces or in combustion furnaces in which the charge is in a container and not in direct contact with the furnace gases, I add to the 25 furnace or to the container, carbon monoxide or a supply of carbon and oxygen from which carbon monoxide may be generated, in order to obtain a reduction of the lithium oxide in accordance with the foregoing equation.

30      It is to be understood that silver alloys may be used in place of pure silver and that such elements as nickel, copper, tin, zinc and other suitable alloying elements, as previously indicated, may be included in minor amounts in the composition to produce desirable variations in the physical properties of the alloy and such alloys of silver are intended to be included under the term "silver" when used in the claims.

The term "alloy" is used throughout the specification and in the claims, in a broad sense, to 40 include a solid solution, mechanical mixture or other form of combination of the various elements thereof.

It is to be understood that these particular examples given of silver-lead-lithium alloys and the 45 procedure for producing the same are to be considered in an illustrative sense and not as defining the limits of the invention.

What I claim is:

50      1. The method of forming an alloy composed at least in part of silver and lead which comprises heating the constituents of the alloy together in a molten state in the presence of lithium until agitation of the molten metal occurs.

55      2. The method of forming an alloy composed at least in part of silver and lead which comprises heating the constituents of the alloy together in a molten state in the presence of lithium until agitation of the molten metal occurs and 60 pouring the molten mass into molds while agitation is continuing.

3. The method of producing agitation in an alloy composed of silver and lead which comprises heating the metals together in a molten state 65 with lithium and simultaneously providing a lithium containing atmosphere about the molten metal.

4. The method of forming an alloy composed at least in part of silver and lead which comprises heating together silver and lead in a 70 molten state in the presence of lithium vapor until agitation of the metal occurs.

5. The method of producing alloys composed at least in part of silver and lead which 75 comprises heating the metals together in a molten

state, agitating the molten mass and continuing the agitation during cooling and up to the point of solidification of the alloy, the agitation being produced by the presence of lithium in contact with the melt.

6. The method of producing silver-lead-lithium 5 alloys which comprises melting together silver, lead and lithium to a temperature at which agitation of the mass occurs and preventing escape of at least part of the lithium from the molten 10 metal.

7. The method of producing silver-lead-lithium anti-friction articles comprising melting silver, 15 lead and lithium together at a temperature sufficient to produce agitation of the molten metal, casting the metal into ingots, remelting the same as desired to a temperature sufficient to cause reagitation and recasting the same into said articles.

8. The method of producing anti-friction al- 20 loys, comprising heating silver and lead in a molten state together with a fractional per cent of lithium and minor proportions of iron, nickel, silicon or tin, until agitation of the molten metal occurs.

9. A silver-lead-lithium alloy containing 5% to 70% lead, not over about 1% of lithium and substantially all of the remainder silver, the lithium being present in sufficient amount to render the 25 alloy substantially homogeneous.

10. A silver-lead-lithium alloy containing 5% to 70% lead in finely divided form, not over about 1% of lithium and substantially all the remainder silver, the lithium being present in sufficient amount to cause substantially uniform dispersion 35 of the lead in the silver.

11. The method of producing silver-lead alloys comprising heating said silver and lead in a molten state in a furnace, and providing lithium in the furnace atmosphere during the heating of 40 the alloy.

12. The method of producing agitation in an alloy composed of silver and lead which comprises heating the metals together in a molten state and providing an atmosphere about the 45 molten metals which exhibits a lithium spectral line.

13. The method of forming an alloy composed at least in part of silver and lead which comprises heating together in a molten state silver 50 and lead in an atmosphere which exhibits a lithium spectral line and maintaining such atmosphere substantially throughout the process.

14. The method of producing a silver-lead 55 lithium alloy comprising heating silver and lead in a molten state in an atmosphere containing lithium produced by the decomposition of a lithium compound.

15. The method of producing a silver-lead- 60 lithium alloy comprising heating silver and lead in a molten state in an atmosphere containing lithium produced by the decomposition of a lithium halide.

16. The method of producing a silver-lead- 65 lithium alloy comprising heating silver and lead in a molten state in an atmosphere containing lithium produced by the decomposition of lithium carbonate.

17. A silver-lead-lithium alloy containing from 70 5% to 70% lead, detectable amounts up to 1% of lithium and substantially all of the remainder silver, the lead being finely distributed within the grains of the silver.